

## UNITED STATES PATENT OFFICE.

NOAK VICTOR HYBINETTE, OF WILMINGTON, DELAWARE.

## HEAT-RESISTING ALLOY AND STRUCTURE.

No Drawing.

Application filed February 2, 1924. Serial No. 690,306.

This invention relates to heat resisting alloys and structures. More particularly, it relates to alloys and structures which are extraordinarily rigid under a heavy load at 5 high temperatures, and also to structures possessing a lesser degree of rigidity combined with some machinability.

In prior applications I have described heat resisting alloys containing approximately 30 10 to 40% nickel, about 15% chromium, and the rest mainly iron, with small additions of deoxidizing agents such as carbon, silicon, manganese, aluminum, magnesium, etc., some of these deoxidizing agents remaining in 15 the alloy and some being removed to a greater or less extent by the deoxidizing action which they exert. Such alloys are suited for wire, sheets, and ordinary castings such as heat treating containers, etc.

20 There exists, however, a demand for heat enduring metallic structures which have the peculiar property of being extraordinarily rigid, even under a heavy load, at temperatures ranging from around 1500 to around 25 2000° F. The present invention is designed to fill such a demand. The invention is also designed to fill the demand for less rigid structures possessing some machinability.

I have discovered that a comparatively 30 large amount of carbon, together with a small amount of aluminum will make low percentage chrome-nickel iron alloys heat enduring; such alloys being below the limits of heat resistance without such addition of 35 carbon and aluminum. This discovery allows me to produce heat enduring alloys of novel composition and with novel properties.

The new alloys of the present invention contain the following ingredients in approximately the following proportions:

40 Nickel from about 5 to about 10%.  
Chromium from about 15 to about 25%.  
Carbon from about 1 to about 2%.  
Aluminum from about 1/2 to about 2%.

45 The remainder mainly iron.  
Such alloys, without the carbon and aluminum in amounts such as indicated, would not be particularly heat resisting; but when carbon and aluminum are both present in 50 proper amount, and when the other ingredients are properly proportioned, the alloy is not only heat resisting but structures made therefrom have the valuable property of rigidity under a heavy load at high temperatures.

55 The aluminum content of the alloy can

be increased several percent, but such increase does not correspondingly increase the strength, and may cause trouble in casting, and, in general, the aluminum should not 60 be increased materially above the amounts indicated. A lowering of the carbon content below the approximate limit indicated causes a considerable lowering in the stiffness of the castings. The lowering of the nickel 65 content tends to cause brittleness at ordinary temperatures while the increase of the nickel content tends to cause toughness and ductility instead of rigid stiffness. At about 10% nickel, the alloy possesses some machinability, e. g. with an emery wheel or chipping tool. Higher proportions of nickel do not 70 produce correspondingly better qualities. A higher percentage of carbon increases machinability. Carbon below 1 1/2 or over 2% 75 decreases heat endurance and strength. At 2% carbon and 10% nickel the alloy still has high heat endurance and fair strength, but the extreme rigidity or high elastic limit and high modulus of elasticity are sacrificed for 80 a fair degree of machinability. Such alloy is suitable for heat treatment containers, etc. For highest strength 6-7% nickel and 1 1/2% carbon and 3/4% aluminum are recommended. Chromium should be held at 18- 85 20%. Lower chromium decreases both heat endurance and strength. Higher chromium gives no corresponding benefit. The silicon content does not appear to be of particular importance so long as the silicon is below 90 about 1%, e. g. around 0.75%, and the amounts of silicon commonly found in the iron from which the alloy is made will ordinarily be such that it does not require to be increased or decreased in amount. Manganese may be present in small amount but if present in too large an amount it has a 95 toughening effect and tends to decrease or destroy the desired rigidity and stiffness. When increased nickel is used in the alloy, 100 an increased amount of aluminum will ordinarily be required, but since a high content of aluminum tends to interfere with casting in sand molds, the nickel and aluminum contents should for best results be kept 105 sufficiently low to avoid such interference.

I have found that a particularly advantageous composition of the alloy for making castings which are rigid at high temperatures is about 20% chromium, about 7% nickel, about 1% aluminum, about 1 1/2% carbon, up to about 1% silicon, up to about 110

$\frac{1}{2}\%$  manganese and the remainder mainly iron. Castings made of this alloy are so hard at ordinary temperatures that they can be worked only with great difficulty with 5 an emery wheel. It is also practically impossible to cut such an alloy with a welding torch. It is therefore unusually well suited for use in safes and similar uses as well as for heat enduring structures.

10 Such an alloy at a temperature of about  $1500^{\circ}$  F. has been found to have an elastic limit of about 8,000, a tensile strength of about 35,000, and a modulus of an elasticity of about 9,000,000. So far as I am aware 15 no other commercially known alloy has such properties.

The alloy is of more or less general use where heat enduring alloys are desired and particularly where castings are desired 20 which have great rigidity under a heavy load at high temperatures. It is not so well adapted, on account of its great hardness, for use in certain high temperature structures where alloys with higher nickel 25 content, and increased toughness and ductility, rather than great rigidity, are more valuable.

The alloy can be cast in the ordinary way 30 in sand molds, and castings of various kinds can be made for use in furnaces and furnace structures. Structures such as I-beams, and other structures for oil stills are particularly valuable when made of the new alloy, since such structures possess great rigidness under 35 a heavy load at high temperature.

The new alloys are relatively inexpensive 40 to manufacture because of their low nickel content, but they nevertheless possess particularly valuable properties of the character referred to.

I believe that I am the first to discover 45 that an alloy of the contents hereinbefore specified of chromium and nickel, which otherwise would not be heat resisting to any practical extent, can be made so by adding a considerable amount of carbon and aluminum at the same time. I also believe that 50 I am the first to discover that such an alloy is particularly suitable for structures where rigidness under a heavy load is wanted at high temperatures.

It will be evident that small additions of many other metals and substances can be added to the alloy without materially chang-

ing the properties thereof, and in some cases 55 with an improvement in the desirable properties of the alloy and of the structures made therefrom.

The new alloys and castings can be produced at a moderate expense, permitting 60 them to be used commercially in large installations where rigidity at high temperatures is desired.

I claim:

1. An alloy which is heat resisting at high 65 temperatures containing the following ingredients in approximately the following proportions: nickel from about 5 to about 10%, chromium from about 15 to about 25%, carbon from about 1 to about 2%, aluminum 70 from about  $\frac{1}{2}$  to about 2%, the remainder mainly iron.

2. An alloy which is heat resisting at 75 high temperatures containing the following ingredients in approximately the following proportions: chromium about 18 to 20%, nickel about 6 to 7%, aluminum about  $\frac{3}{4}$  to 1%, carbon about  $1\frac{1}{2}\%$ , the remainder mainly iron.

3. An alloy having approximately the following composition:—about 20% chromium, about 7% nickel, about 1% aluminum, about  $1\frac{1}{2}\%$  carbon, and the remainder mainly iron, said alloy having approximately the 85 following properties at a temperature of about  $1500^{\circ}$  F. namely, an elastic limit of about 8,000, a tensile strength of about 35,000 and a modulus of elasticity of about 9,000,000.

4. A cast structure made of an alloy of 90 the composition specified in claim 1.

5. A cast structure made of an alloy of the composition specified in claim 2, said cast structure possessing great rigidness under a heavy load at temperatures ranging 95 from about  $1500^{\circ}$  to about  $2000^{\circ}$  F.

6. Cast I-beams and other structural shapes made of an alloy such as specified in claim 1, said cast structures being characterized by great rigidity at high temperatures. 100

7. Cast I-beams and other structural shapes made of an alloy such as specified in claim 2, said cast structures being characterized by great rigidity at high temperatures. 105

In testimony whereof I affix my signature.

NOAK VICTOR HYBINETTE.